

## UNITED STATES PATENT OFFICE

ORIN D. CUNNINGHAM, OF INDIANAPOLIS, INDIANA, ASSIGNOR TO PETER C. REILLY,  
OF INDIANAPOLIS, INDIANA

## PROCESS OF ORE FLOTATION AND FLOTATION REAGENT

No Drawing.

Application filed February 19, 1931. Serial No. 517,126.

This invention relates to the concentration of materials, particularly metalliferous materials by the froth flotation operation, and has for its object the provision for certain improvements involving the use of a certain class of organic substances as collecting agents in the concentration of such materials as ores and minerals. The invention embraces both the product and the method of making the same, as well as the use of the product in the froth flotation operation.

The present invention is based on the discovery that certain unsaturated fatty acid compounds such as, for example, oleic acid dissolved in or mixed with a phenol (or certain other substances herein classified as phenol equivalents), when reacted on with a phosphorus sulfur compound such as, for example, phosphorus pentasulfide ( $P_2S_5$ ), become chemically transformed to what will herein be termed "thiophospho-fatty acid compounds", which compounds are highly active as flotation collecting agents.

It is pointed out that in the above reaction the phenol or its equivalent is involved in the transformation of an unsaturated fatty acid substance to a thiophospho-fatty acid compound, said compound containing the phenols, etc. as a part of its molecular structure.

Although oleic acid has been indicated as preferred unsaturated fatty acid substance for preparing the flotation reagent of the present invention, other unsaturated fatty acids, (containing 4—22 carbon atoms), or mixtures of the same can also be employed, such as, for example, crotonic acid, decylenic acid, undecylenic acid, elaidic acid, rapic acid, ricinoleic acid, linoleic acid, brassidic acid, eruic, etc.

Or instead of an unsaturated fatty acid the unsaturated fatty acid esters may be employed, such as, for example, butyl oleate. Of interest also are the unsaturated fatty acid substances which consist essentially of glyceride esters of the unsaturated fatty acids such as, for example, olive oil, fish oils, cotton-seed oils, tung oil, etc. While these will function they are not as active as the unsaturated fatty acids.

As phenol equivalents that may be employed in the preparation of the thiophospho-fatty acid compounds of the present invention, we give the following classification of compounds:

(a) Phenolic compounds, such as carbolic acid, cresols, xylenols, tar acids or closely related homologues of the same.

(b) The hydrogenated phenolic compounds.

(c) The aliphatic alcohols, containing from one up to six carbon atoms such as, for example, ethyl alcohol, n-propyl alcohol, n-butyl alcohol, n-amyl alcohol, n-hexyl alcohol, as well as isomers of these alcohols.

(d) The aliphatic and aromatic mercaptols such as the ethyl, propyl, etc. mercaptols, phenyl mercaptol or closely related homologues of the same.

(e) The aliphatic and aromatic amines such as for example, ethyl amine, aniline, toluidine, alpha-naphthyl-amine or closely related homologues.

Bodies falling within the above classification (a to e inclusive) include phenols and substances which are, in the present invention, equivalents of phenols. These substances may be referred to generically as "a phenol-like substance", which term is herein-after used in that sense.

It is understood that any mixtures of the above classified compounds may also be employed, such mixtures being considered as phenol equivalents and such mixtures are included within the scope of the present invention.

The thiophospho-fatty acid compounds prepared by the reaction of  $P_2S_5$  on the unsaturated fatty acid substance dissolved or mixed with a phenol or phenol equivalent, constitute a class of flotation reagents that possess high collecting activity toward minerals and metalliferous materials in the froth flotation operations; particularly are they effective toward so-called oxidized ores, that is, ores containing some non-sulfide minerals such as for example, carbonates, basic carbonates, oxides, silicates, etc.

It is not necessary that chemically pure substances be used in the preparation of the

55

65

80

85

90

95

100

above reagents, since unrefined products can be employed with metallurgical results practically as good as those obtained with pure chemicals.

5 The following example is illustrative of the preparation of the flotation reagent of the present invention:

To a mixture of 50 parts of oleic acid and 50 parts of a phenol at 100° C., 20 parts of 10  $P_2S_5$  are slowly added with stirring. After all of the  $P_2S_5$  has been added the reaction is continued for about three hours.

Working under substantially the same conditions, the phenol in the above preparation 15 may be replaced with an equal weight (50 parts, or thereabout) of any of the various phenol equivalents listed above, or in place of oleic acid, other unsaturated fatty acid substances as above indicated may be employed. Phosphorus trisulfide may be used 20 instead of the pentasulfide in the example given, being employed in equimolecular proportion under very much the same reaction conditions.

25 In the above preparation I do not limit myself to the reaction temperature given, nor to the proportion of reacting materials employed. In some cases a reaction temperature of 50° C., or thereabout, and a longer 30 reaction period may advantageously be employed, while in other cases a temperature of 150° C., or thereabout, is preferable. It is conceivable that even lower or higher temperatures than those given may be more suitable 35 for certain of these reactions.

Instead of carrying out the reaction as above indicated, the reaction may be carried out in two steps, first the reaction of phenol (or its equivalent) with  $P_2S_5$  to form an organic thiophosphoric acid, which is then combined with oleic acid, as the second step, to form a thiophospho-oleic acid compound. Either procedure yields substantially the same reaction product.

45 Without limiting the present invention to any theory of reaction, it is believed that the reactions involved in the above type of preparation include first the formation of an intermediate organic thiophosphoric acid 50 which then reacts with oleic acid, for example, at the double bond to form a thiophospho-oleic acid reaction product.

Where an unsaturated fatty acid is employed, as in the above example, the reaction 55 product may be reacted with an alkali or alkaline earth hydroxide to form the alkali or alkaline earth metal salt of the thiophospho-fatty acid compound, which with some ores 60 may be a preferable reagent to the free acid compound.

In the froth flotation of ores by the use of the above products as collecting agents the 65 said products, although possessing some frothing action, may require the use of a suitable frothing agent such as, for example,

pine oil, terpineol, cresylic acid or the like. The said reagents and frothing agents may be introduced into the ore pulp in any convenient manner and at any appropriate stage preceding or during the flotation operation. 70 Thus, for example, it may be mixed with the ore pulp in a tube mill or other device in which the ore is being prepared; and the amount of said reagent may be varied between wide limits depending upon the nature 75 of the ore under treatment. Good results are obtained in many cases by the use of 0.1 to 0.2 pound per ton of ore.

The pulp is then subjected to the ordinary aeration or froth flotation operation, producing a foam carrying the mineral content from the ore. The flotation can be conducted in any type of froth flotation cell and in a neutral, alkaline or acid circuit, as desired.

In the use of an alkaline circuit it is sometimes preferable to add the alkali after the above reagents have been added and thoroughly dispersed with the ore pulp.

As illustrative of the practice of the invention 0.15 pound per ton of a thiophospho-oleic acid compound (made by the reaction of oleic acid, pentasol (a mixture of isomeric alcohols containing 5 carbon atoms), and  $P_2S_5$ ), was employed in conjunction with the froth flotation of a difficultly floatable copper bearing mineral (containing about 23% oxidized copper mineral) of the Phelps-Dodge Corporation, together with 0.1 pound of terpineol, an alkaline circuit being employed therewith. A recovery of 100 80%, or thereabout, of the copper bearing mineral was obtained, in the form of a good grade concentrate.

This same reagent when employed in conjunction with the flotation concentration of 105 Utah Copper Co. ore, under substantially the same conditions, gave a recovery of better than 90% of the copper bearing mineral together with a good grade of concentrate.

In the above tests the thiophospho-oleic 110 acid reagent was first thoroughly dispersed with the ore pulp in a ball mill before adding the lime for alkalinity.

What is claimed is:

1. A process which comprises floating ore 115 material in the presence of a reaction product of a phosphorus sulfide on an unsaturated fatty acid substance and a phenol-like substance, as herein specified.

2. The froth flotation of metalliferous material while in the presence of a reaction product of a phosphorus sulfide on an unsaturated fatty acid substance and a phenol-like substance, as herein specified.

3. The froth flotation of metalliferous material while in the presence of a reaction product of a phosphorus sulfide on an unsaturated fatty acid, containing 4-22 carbon atoms, and a phenol-like substance, as herein specified.

4. The froth flotation of metalliferous material while in the presence of a reaction product of a phosphorus sulfide on oleic acid and a phenol-like substance, as herein specified.
5. The froth flotation of metalliferous material while in the presence of a reaction product of a phosphorus sulfide on oleic acid and a tar acid, as herein specified.
- 10 6. The froth flotation of metalliferous material while in the presence of a reaction product of a phosphorus sulfide, on oleic acid and an alcohol, as herein specified.
- 15 7. The froth flotation of metalliferous material while in the presence of a reaction product of a phosphorus sulfide on oleic acid and pentasol, as herein specified.
- 20 8. The froth flotation of metalliferous material while in the presence of a reaction product of a phosphorus sulfide such on oleic acid and an organic amino compound, as herein specified.
- 25 9. A new flotation reagent comprising a reaction product of a phosphorus sulfide on an unsaturated fatty acid substance and a phenol, as herein specified.
- 30 10. A new chemical product comprising a reaction product of a phosphorus sulfide on an unsaturated fatty acid substance and a phenol, as herein specified.
- 35 11. A process which comprises reacting with a phosphorus sulfur compound on an unsaturated fatty acid substance and a phenol to yield a thiophospho-fatty acid compound of flotation value, as herein specified.
- 40 12. In the art of froth flotation, the step of floating material to be concentrated in the presence of the herein described flotation agent which comprises a reaction product of a phosphorus sulfide compound on an unsaturated fatty acid substance and a substance selected from the herein described group consisting of (a) phenolic compounds,
- 45 (b) the hydrogenated phenolic compounds, (c) the aliphatic alcohols containing from 1 to 6 carbon atoms, (d) the aliphatic and aromatic mercaptols, and (e) the aliphatic and aromatic amines.
- 50 13. In the art of froth flotation the step of floating material to be concentrated in the presence of the herein described flotation agent which comprises a reaction product of a phosphorus sulfur compound on an unsaturated fatty acid substance and a phenol.
- 55 14. In the art of froth flotation the step of floating material to be concentrated in the presence of the herein described flotation agent which comprises an alkali-forming metal salt and a thiophospho-fatty acid compound.
- 60 15. In the art of froth flotation the step of floating material to be concentrated in the presence of the herein described flotation agent which comprises a sodium salt of a thiophospho-fatty acid compound.
16. The froth flotation of ore material in the presence of a reaction product of  $P_2S_5$  on an unsaturated fatty acid substance and a phenol-like substance.
17. The froth flotation of metalliferous material in the presence of a reaction product of  $P_2S_5$  on an unsaturated fatty acid substance and a phenol-like substance.
18. In the art of froth flotation the step of floating material to be concentrated in the presence of the herein described flotation agent which comprises a reaction product of a phosphorus sulfur compound on an unsaturated fatty acid substance and a phenol-like substance.
- In testimony whereof I have signed my name to this specification.
- ORIN D. CUNNINGHAM.
- 85
- 90
- 95
- 100
- 105
- 110
- 115
- 120
- 125
- 130

**CERTIFICATE OF CORRECTION.**

**Patent No. 1,902,838.**

**March 28, 1933.**

**ORIN D. CUNNINGHAM.**

**It is hereby certified that error appears in the printed specification of the above numbered patent requiring correction as follows: Page 3, line 20, claim 8, strike out the word "such"; and that the said Letters Patent should be read with this correction therein that the same may conform to the record of the case in the Patent Office.**

**Signed and sealed this 16th day of May, A. D. 1933.**

**(Seal)**

**M. J. Moore.  
Acting Commissioner of Patents.**